

# United States Patent Office

3,169,858

Patented Feb. 16, 1965

1

3,169,858

## AUSTENITIC STEEL ALLOY

Gerald B. Heydt, Reading, and Clyde Raymond Whitney, Wyoming, Pa., assignors to The Carpenter Steel Company, Reading, Pa., a corporation of New Jersey  
No Drawing. Filed May 24, 1962, Ser. No. 197,290

5 Claims. (Cl. 75—124)

This invention relates to an austenitic iron base alloy which is age hardenable and more particularly to such an alloy having high strength at elevated temperatures.

This application in part is a continuation of our pending application filed on January 23, 1961, Serial No. 83,895, and assigned to the assignee of the present application.

Hitherto, for use where high strength at elevated temperature had been required austenitic iron base alloys were provided having a composition balanced so as to respond to an aging or precipitation hardening treatment. More particularly such alloys were balanced so that upon aging they underwent a precipitation hardening and strengthening mechanism such that a precipitate was formed having a lattice structure the same as that of the alloy matrix in which it is formed and also having a lattice parameter which is close to but yet constitutes a misfit with the lattice parameter of the matrix.

The present invention is particularly concerned with improving those iron base austenitic precipitation hardening alloys which harden during aging by a mechanism involving the formation of a face centered cubic precipitate known as "gamma prime." The usefulness of such alloys has been limited by the fact that the gamma prime precipitate transformed during use at elevated temperature after a relatively short time so that the composition lost its strength. This transformation results from the fact that the gamma prime, face centered cubic structure formed in the original aging treatment underwent a further transformation to a hexagonal close packed structure, known as "eta phase." The extent of the transformation depends upon the duration of the exposure to temperatures between about 1100° F. to 1700° F. and the degree of stress to which the part formed of the alloy is subjected.

In the absence of stress at about 1400° F., the transformation of the face centered cubic to the hexagonal close packed structure is apparent in as little as sixteen hours and after about one hundred hours the transformation has progressed to such an extent that the part formed of the alloy has insufficient strength for its intended use. The transformation of the face centered cubic gamma prime phase to the hexagonal close packed structure proceeds more rapidly at any given temperature between about 1100° F. and 1700° F. as the part is subjected to greater stress. Thus, in service where the parts formed of such alloys are subjected to stress at elevated temperature, they have been found to have an objectionably short useful life.

While some measure of success has been achieved heretofore in providing such alloys having good strength at elevated temperatures for periods of about one hundred hours as represented by stress rupture tests, such alloys have left much to be desired insofar as their stress rupture ductility was concerned. For example, such alloys were considered to be unduly prone to failure when subjected to stress at high temperature after having been scratched or notched.

It is therefore a principal object of the present invention to provide an age hardening austenitic iron base alloy characterized by high strength, high stress rupture ductility and longer useful life under stress at elevated temperatures up to about 1500° F. by means of the formation of a gamma prime precipitate which has enhanced stability against transformation to the undesired eta phase.

The alloy of the present invention is particularly well

2

suit for use in forming such parts as wheels and rings for use in jet engines. Thus, the alloy of the present invention is not only characterized by high strength and stress rupture ductility at elevated temperatures but also is characterized by good resistance to oxidation and corrosion at such temperatures.

A more specific object of the present invention is to provide such an alloy which may be readily melted and cast into ingots that may be economically hot worked and formed into parts.

We have discovered that the foregoing objects can be achieved with an austenitic steel having the following analysis in percent by weight within the tolerances of good commercial melting practices:

|    |                            |                     |
|----|----------------------------|---------------------|
| 15 | Carbon                     | Up to .10% maximum. |
|    | Manganese                  | Up to 2%.           |
|    | Silicon                    | Up to .25% maximum. |
|    | Chromium                   | 14% to 20%.         |
|    | Nickel                     | 20% to 30%.         |
| 20 | Molybdenum and/or tungsten | 1% to 3%.           |
|    | Vanadium                   | .10% to 1.0%.       |
|    | Aluminum                   | .75% to 1.75%.      |
|    | Titanium                   | 2.75% to 3.75%.     |
| 25 | Boron                      | .003% to .025%.     |

the balance being principally all iron except for incidental impurities such as phosphorous, sulfur, nitrogen, oxygen and the like, the ratio of the titanium content to the aluminum content being at least equal to about 2.

30 The proper balance of the alloying elements of this composition is highly critical and must be carefully maintained if sound steel having the required properties at temperatures as high as 1500° F. is to be obtained suitable for such use as in the fabrication of jet engine parts.

35 In this alloy, the maximum carbon content must not exceed about .10% and is preferably maintained at a much lower level below about .05% maximum. Vanadium is included in this composition in amounts ranging from about .10% to 1% primarily to tie up the carbon and prevent the formation of a titanium carbide. When the carbon content is maintained below .05%, then only about .15% to .3% vanadium is required for this purpose. Manganese may be present in amounts up to about 2% but is preferably limited to no more than .25%.

40 Silicon when present in more than very small amounts results in the formation of unsound areas in forged billets formed from relatively large commercial ingots because of the formation of a nickel-titanium-silicide segregate believed to be  $Ni_{13}Ti_8Si_6$  identified as G phase. Therefore, silicon is limited to no more than about .25% as is brought out in said application Serial No. 83,895. Preferably, the silicon content is maintained below .15% in order to ensure obtaining the soundest steel.

45 Small additions of boron work to improve the rupture strength of our alloy at elevated temperatures. For this purpose, from about .003% to .025% boron provides good results. When present in amounts above .025%, boron tends to form borides, particularly with nickel, and this has a detrimental effect upon the forgeability and mechanical properties of the alloy. Preferably, lower amounts below .013% boron are utilized to provide optimum results.

50 Chromium and nickel form the major portion of the alloying additions in our alloy. From about 14% to 20% chromium provides the required degree of oxidation and corrosion resistance. Because chromium is a relatively strong ferrite former, preferably about 15% to 17% chromium is utilized in this composition. Nickel not only tends to favor the formation of austenite but also takes part in the aging mechanism by which the present alloy is strengthened. While from 20% to 30% nickel is

desirable, we preferably utilize from about 25 to 27% nickel to ensure a fully austenitic alloy and at the same time provide sufficient nickel for the precipitation and hardening reaction.

Molybdenum and/or tungsten are included because they improve the high temperature strength of the alloy. For this purpose, molybdenum and tungsten are generally equivalent and either or both may be included to provide a total addition ranging from about 1% to 3%. Best results are achieved when molybdenum is utilized alone and preferably in an amount ranging from about 1.25 to 1.75%.

Titanium largely contributes to the rupture strength and the tensile strength of the alloy and for this purpose about 2.75% to 3.75% titanium is utilized. When titanium is present in an amount less than about 2.75% both the high room temperature tensile strength and the high rupture strength at elevated temperatures characteristic of our alloy are not attainable. Larger amounts of titanium than about 3.75% tend to impair the hot workability of the composition. Titanium, in the absence of at least about .75% aluminum, reacts with nickel during aging to provide a gamma prime phase identified as  $Ni_3Ti$  which has less stability than desired against transformation to the undesired eta phase.

We have unexpectedly discovered that when aluminum is present in our alloy in amounts varying from about .75% to 1.75%, the more stable gamma prime phase is formed on aging identified as  $Ni_3(TiAl)$ , most consistent results being attained when aluminum is present in an amount varying from 1% to 1.5%. Our experiments have shown that the improved stress rupture ductility and improved strength at elevated temperatures as high as 1500° F. is brought about by the presence in our alloy of the critically related proportions of the titanium and aluminum contents. It is essential to the achievement of improved high temperature stress rupture ductility not only without a loss in high temperature strength but with an improved high temperature strength that, at any level within the stated limits, the titanium content be sufficiently greater than the aluminum content so as to ensure the degree of misfit between the lattice parameters of the gamma prime phase and the alloy matrix required in strengthening the alloy. However, the degree of misfit must not be so great as to cause weakening rather than strengthening of the alloy. We have found that when the aluminum content is too close to, equal to, or greater than the titanium content, the resulting misfit between the lattice structures is excessive and results in a composition having low strength at high temperature. Best results have been achieved when at any level of titanium within the limits stated, the ratio of the percent by weight content of titanium to that of aluminum is at least equal to about 2.5. When the value of this ratio is decreased below about 2.5 by increasing the amount of the aluminum in relation to the titanium, the high temperature strength of our alloy is affected and when the ratio is less than about 2, the improved high temperature strength of our alloy is not obtained.

Thus, the alloy which we have produced with preferred results has the following composition in percent by weight within the tolerances of good commercial melting practice:

|            |                     |
|------------|---------------------|
| Carbon     | Up to .05% maximum. |
| Manganese  | Up to .25% maximum. |
| Silicon    | Up to .15% maximum. |
| Chromium   | 15% to 17%.         |
| Nickel     | 25% to 27%.         |
| Molybdenum | 1.25% to 1.75%.     |
| Vanadium   | .15% to .30%.       |
| Aluminum   | 1% to 1.5%.         |
| Titanium   | 3% to 3.5%.         |
| Boron      | .003% to .013%.     |

the ratio of the titanium content to the aluminum content

being at least 2.5 and the balance being principally all iron except for incidental impurities.

Our alloy is readily prepared and worked in accordance with good standard commercial practices. No special heat treatment is required. Solution treatment at about 1800° F. to 1900° F. for about one to two hours followed by oil or air quenching and an aging or precipitation hardening treatment at about 1300° F. to 1500° F. for about sixteen hours provides good results.

As a specific example of our alloy an ingot was melted and cast containing .021% carbon, .21% manganese, .21% silicon, 14.40% chromium, 26.16% nickel, 1.12% molybdenum, .28% vanadium, 1.34% aluminum, 3.31% titanium, .010% boron and the balance all iron except for incidental impurities. The ingot was hot worked to half inch bars, then solution treated and aged. In this instance the solution treatment was carried out at 1900° F. for two hours followed by quenching. A hardness of Rockwell C 34 was obtained after aging for sixteen hours at 1400° F. followed by cooling in air as compared to an as-solution-treated and quenched hardness of Rockwell B 76. When a specimen of this alloy was aged for four hours at 1500° F. it showed a hardness of Rockwell C 33/34 and when aged for twenty hours at that temperature a hardness of Rockwell C 32 was still obtained.

The aged bars were machined to form standard combination smooth-notch stress rupture specimens having a smooth section .195 inch in diameter and a gauge length of .780 inch merging with a thicker section .275 inch in diameter in which a circular notch was formed having a .195 inch diameter at the root of the notch, a root radius of .005 inch and a notch angle of 60°. At 1300° F., a stress load of 62,000 p.s.i. was sustained for eighty hours before rupture with a 17% elongation and 25% reduction in area. The failure occurred in the smooth portion of the test specimen and not at the notch, indicating that the alloy has good stress rupture ductility.

On the other hand, tests carried out on similarly prepared specimens but not containing titanium and aluminum in the stated ratio showed significantly lower attainable as-aged hardness as well as indications of over-aging when aged for sixteen hours at 1400° F. While such specimens showed good stress rupture ductility, they were characterized by poor stress rupture strength. For example, an alloy having essentially the analysis of the specific example given above but containing 2.38% aluminum and 1.93% titanium was ruptured in the smooth area of the specimen after only seven hours when subjected to a stress of 62,000 p.s.i. at 1300° F. with a 27% elongation and 32% reduction in area. For further comparison, it may also be noted that the last mentioned alloy when aged at 1400° F. for sixteen hours had a hardness of only Rockwell C 28 and when aged for four hours at 1500° F. was over-aged to such an extent that it had a hardness of only Rockwell B 97.

The terms and expressions which have been employed are used as terms of description and not of limitation, and there is no intention, in the use of such terms and expressions of excluding any equivalents of the features shown and described or portions thereof, but it is recognized that various modifications are possible within the scope of the invention claimed.

We claim:

1. An age hardening austenitic iron base alloy which in its hardened condition has good strength and ductility at temperatures up to above 1500° F., which is essentially free of a silicon-bearing segregate phase and which within the tolerances of good melting practice consists essentially of up to .10% carbon, up to 2% manganese, up to .25% silicon, 14% to 20% chromium, 20% to 30% nickel, 1% to 3% molybdenum, 2.75% to 3.75% titanium, .75% to 1.75% aluminum, .10% to 1.0% vanadium, .003% to .025% boron, the titanium content being sufficiently greater than the aluminum content to limit the extent of the misfit between the lattice parameter of the gamma

prime phase and that of the alloy matrix when aged, and the remainder essentially iron.

2. An age hardening austenitic iron base alloy which in its hardened condition has good strength and ductility at temperatures up to about 1500° F., which is essentially free of a silicon-bearing segregate phase and which within the tolerances of good melting practice consists essentially of up to .10% carbon, up to 2% manganese, up to .25% silicon, 14% to 20% chromium, 20% to 30% nickel, 1% to 3% molybdenum, 2.75% to 3.75% titanium, .75% to 1.75% aluminum, .10% to 1.0% vanadium, .003% to .025% boron, the ratio of the titanium content to the aluminum content being about equal to at least 2, and the remainder essentially iron.

3. An age hardening austenitic iron base alloy which in its hardened condition has good strength and ductility at temperatures up to about 1500° F., which is essentially free of a silicon-bearing segregate phase and which within the tolerances of good melting practice consists essentially of up to .10% carbon, up to 2% manganese, up to .25% silicon, 14% to 20% chromium, 20% to 30% nickel, 1% to 3% molybdenum, 2.75% to 3.75% titanium, .75% to 1.75% aluminum, .10% to 1.0% vanadium, .003% to .025% boron, the ratio of the titanium content to the aluminum content being about equal to at least 2.5, and the remainder essentially iron.

4. An age hardening austenitic iron base alloy which

in its hardened condition has good strength and ductility at temperatures up to about 1000° F., which is essentially free of a silicon-bearing segregate phase and which within the tolerances of good melting practice consists essentially of up to .05% carbon, up to .25% manganese, up to .15% silicon, 15% to 17% chromium, 25% to 27% nickel, 1.25% to 1.75% molybdenum, 3% to 3.5% titanium, 1% to 1.5% aluminum, .15% to .30% vanadium, .003% to .013% boron, the ratio of the titanium content to the aluminum content being about equal to at least 2, and the balance essentially iron.

5. An age hardening austenitic iron base alloy which in its hardened condition has good strength and ductility at temperatures up to about 1500° F., which is essentially free of a silicon-bearing segregate phase and which within the tolerances of good melting practice consists essentially of up to .05% carbon, up to .25% manganese, up to .15% silicon, 15% to 17% chromium, 25% to 27% nickel, 1.25% to 1.75% molybdenum, 3% to 3.5% titanium, 1% to 1.5% aluminum, .15% to .30% vanadium, .003% to .013% boron, the ratio of the titanium content to the aluminum content being about equal to at least 2.5, and the balance essentially iron.

References Cited in the file of this patent

UNITED STATES PATENTS

2,750,283 Loveless ----- June 12, 1956

UNITED STATES PATENT OFFICE  
CERTIFICATE OF CORRECTION

Patent No. 3,169,858

February 16, 1965

Gerald B. Heydt et al.

It is hereby certified that error appears in the above numbered patent requiring correction and that the said Letters Patent should read as corrected below.

In the grant, line 1, for "Gerald B. Heyst" read  
-- Gerald B. Heydt --; column 5, line 14, for "essenially"  
read -- essentially --; column 6, line 2, for "1000° F." read  
-- 1500° F. --.

Signed and sealed this 17th day of August 1965.

(SEAL)

Attest:

ERNEST W. SWIDER  
Attesting Officer

EDWARD J. BRENNER  
Commissioner of Patents